

## UNITED STATES PATENT OFFICE

WILLIAM F. RICHTER, OF APOLLO, PENNSYLVANIA, ASSIGNOR TO CHEMICAL HOLDING CORPORATION, OF APOLLO, PENNSYLVANIA, A CORPORATION OF DELAWARE

## MANUFACTURE OF LUSTERLESS RAYON

No Drawing.

Application filed October 28, 1930. Serial No. 491,815.

This invention relates to the fabrication of viscose into useful products, and particularly to the production of permanently lusterless artificial silk.

- 5 The baths commonly used in spinning viscose produce fibers having high surface brilliancy, but the trade demand for artificial silks of decreased luster has led to the development of the so-called "delustered" rayon.  
 10 Various means are used in delustering artificial silk, chiefly by special treatments after spinning, which deaden the luster. The silk produced in this manner, while initially possessing the desired lower luster, gradually  
 15 increases in luster after being used or washed. This characteristic is, of course, objectionable. Spinning baths for the direct production of lusterless rayons have not yet been developed and used commercially, because in  
 20 general such baths are objectionable in that they are of complex composition, and relatively high concentrations of salts are used. Therefore, not only are such baths relatively expensive, but the yarn may be weakened  
 25 through crystallization of salts upon the fibers.

It is among the objects of this invention to provide an improved process of producing lusterless rayon from viscose, in which use  
 30 is made of baths of simple composition, which are easily used, inexpensive, produce permanently lusterless rayon, and which minimize the disadvantages of prior means used for this purpose.

35 The invention is predicated upon my discovery that rayon which is permanently lusterless, and which possesses satisfactory physical characteristics, may be produced by precipitating viscose in a bath consisting of  
 40 sulfuric acid and a soluble nickel salt.

In the practice of this invention viscose is prepared according to any desired procedure, and it is then spun in the usual manner in a bath consisting of sulfuric acid and nickel salt, preferably nickel sulfate in an amount less than the sulfuric acid. Most suitably the bath consists of from about 5 to  
 45 7 per cent of sulfuric acid and about 1.5% to 4.5% of nickel sulfate. Especially desir-

able results are obtained through the use of a bath having the following composition:

|                |    |    |
|----------------|----|----|
| Sulfuric acid  | 6% | 55 |
| Nickel sulfate | 3% |    |

Most suitably the baths provided by this invention are used at somewhat elevated temperatures, for example, from about 30° C. to 45° C. In the preferred embodiment of the invention the bath is maintained at a 60 temperature from about 35° C. to 40° C.

The artificial silk thus produced is characterized by a soft, substantially lusterless appearance, and it retains this lusterless condition permanently. That is, it is apparently 65 impossible to cause it to assume a higher luster by any known procedure. Thus, it does not gain in luster upon repeated washing, or upon prolonged boiling with any of the materials to which it may be subjected in use. 70 Furthermore, the artificial silk produced by the process provided by this invention possesses all of the physical properties which are characteristic of the normal, or glassy rayons.

75 In addition to producing rayon having the characteristics just described, the baths used in the practise of the invention have the advantage that their composition is exceedingly simple and their cost is low. Not only is 80 the salt concentration appreciably lower than that commonly used in rayon spinning baths, but the salt used does not tend to crystallize in the yarn as readily as those commonly used, such as sodium or magnesium sulfates. 85 Therefore, because of these factors weakening of the rayon through crystallization and subsequent washing of the salts is minimized or practically eliminated.

890 Although nickel salts have been recommended previously for use in rayon precipitating baths, such baths have been of the type which produce rayon of high luster. For such purposes cobalt salts are the full equivalent of nickel salts. In the practice of the 95 present invention such equivalency apparently does not hold.

According to the provisions of the patent statutes, I have explained the principle and mode of operation of my invention, and have 100

described what I now consider to represent its best embodiment. However, I desire to have it understood that, within the scope of the appended claims the invention may be practised otherwise than as specifically illustrated and described.

I claim:

1. In a process of preparing permanently lusterless artificial fibers from viscose the step comprising precipitating the viscose in a bath consisting of about 5 to 7 per cent of sulfuric acid, and about 1.5 to 4.5 per cent of nickel sulfate.
- 15 2. In a process of preparing permanently lusterless artificial fibers from viscose the step comprising precipitating the viscose in a bath consisting of about 6 per cent of sulfuric acid, and about 1.5 to 4.5 per cent of nickel sulfate, said bath being maintained at a temperature 20 of about 30 to 45° C.
- 25 3. In a process of preparing permanently lusterless artificial fibers from viscose the step comprising precipitating the viscose in a bath consisting of about 6 per cent sulfuric acid, and about 3 per cent of nickel sulfate.

In testimony whereof, I sign my name.

WILLIAM F. RICHTER.

30

35

40

45

50

55

60

65